# EUROPEAN PATENT SPECIFICATION

(11) **EP 0 576 608 B1**
(45) Date of publication and mention of the grant of the patent: **18.01.1995**
(21) Application number: 92910440.4
(22) Date of filing: 07.05.1992
(51) Int. Cl.: B27K 3/34, B27K 3/52

(54) **METHOD OF QUALITY IMPROVEMENT OF WOODEN ARTICLES, SUCH AS IMPROVED PRESERVATION OF THE WOOD THROUGH IMPREGNATION THEREOF**
VERFAHREN ZUR QUALITÄTSVERBESSERUNG VON HOLZARTIKELN WIE ETWA KONSERVIERUNG DES HOLZES DURCH IMPRÄGNIERUNG
PROCEDE DESTINE A CONFERER UNE MEILLEURE QUALITE A DES ARTICLES EN BOIS, TELLE QU'UNE MEILLEURE PRESERVATION DU BOIS, PAR L'INTERMEDIAIRE DE SON IMPREGNATION

(30) Priority: 07.05.1991 DK 848/91
(43) Date of publication of application: 05.01.1994
(73) Proprietor: SCHIRNIG, Ulrich Herbert, DK-1117 Copenhagen K (DK)
(72) Inventor: SCHIRNIG, Ulrich Herbert, DK-1117 Copenhagen K (DK)
(74) Representative: Noergaard, Tage
(86) International application number: DK9200148
(87) International publication number: WO9219429

(56) References cited:
- FR-A- 397 786
- SE-B- 465 760

## Description

The invention relates to a method of quality improvement of wooden articles such as improved preservation of wood through impregnation thereof, and where the impregnation is carried out by the wooden articles being immersed in a bath of hot linseed oil or similar vegetable oil, heated to at least 110°C, whereby the water present in the wood evaporates and diffuses through the wood and the oil while the hot oil simultaneously penetrates into the pores and cavities of the wood, whereupon the wooden articles are taken out of the bath and the oil oozed in is made to cure and thereby to stiffen the wood.

French patent No. 397,786 disloses a method for drying wood and improving the quality of the wood by immersing said wood into hot linseed oil or similar oils. The temperature of the oil must be sufficiently high for the water in the wood to evaporate and the wood to be impregnated with the oil. It is stated that the temperature is conventionally 100-110°C. This method is not quite satisfactory because the wooden articles tend to be distorted at this relatively low impregnation temperature, as is also the case when drying in hot air.

It is the object of the invention to provide a method of the above type which makes it possible to carry out the desired impregnation without the wooden articles being distorted or displaying cracks or crevices, and which is capable of preventing or destroying a possible insect or fungus attack on the wood.

The method according to the invention is characterised in that during the immersion of the wooden articles, the linseed oil bath has a temperature in the range of 145°-250°C, preferably near 250°C, and that an insecticide and/or fungicide has been added to the linseed oil. As a result, first of all the treated wooden articles do not warp or display cracks or crevices and they are, furthermore, resistant to insect or fungal atacks. By the penetration of the very hot oil the temperature of the wood is increased almost shock-like, whereby its natural or absorbed content of water is suddenly brought above the boiling point and is sweated out. The water is thus replaced by the oil which fills all natural or unnatural cavities of the wood. After a natural or accelerated drying, the oozed in oil cures, thereby stiffening/improving the wood. To this should be added that the treated wooden articles stand mechanical treatment at higher rates of speed than so far known, as the impregnation oil has a considerable lubricating effect. Furthermore, the surface of the wooden articles better stand painting at a later time. Finally, the method is environmentally more acceptable than the known pressure impregnation where salts are used which may be toxinous.

An embodiment of the method according to the invention is characterised in that a drier (siccative) is added to the linseed oil used thereby accelerating the curing of the oil.

A second embodiment of the invention according to the invention is characterised in that colour pigments have been added to the linseed oil used. As a result, the finished wooden articles get a more attractive appearance, as the colour pigments particularly settle on the surface of the wooden articles. The penetration depends on the type of wood, dimension and original place in the stem.

A further embodiment of the method according to the invention is characterised in that the treated articles are of old (previsously used) wood. As a result, old apparently worn out wood may find new use, for instance in connection with a restoration, as the wood gets back its old strength, indeed may get stonger than it naturally was.

According to the invention, the immersion may be carried out for a relatively short period whereby the penetration of the linseed oil in the wooden material takes place to a rather slight depth. Thereby wooden articles of a rather different quality may be obtained.

Furthermore, according to the invention the wooden articles may be subjected to a controlled drying (curing process) in heat chamber or autoclave after the impregnation with the hot linseed oil. It is thereby further ensured that the end product is not crooked.

Moreover, according to the invention the linseed bath may have a temperature of 145-250°C, preferably 175-245°C, during the immersion of the wooden articles, which has been found particularly advantageous.

Further, according to the invention the linseed bath may have a temperature of 210-240°C, preferably 225-235°C during the immersion of the wooden articles, which is also very advantageous.

Finally, according to the invention, the wooden articles may be kept immersed for at least 10 minutes, preferably 15-45 minutes, whereby a suitable oozing in of oil is obtained.

The present method is environmentally acceptable because the substances used are degradable and possible residues may be used for other purposes, for instance paint.

The invention is described in greater details below with reference to the Examples.

### Example 1

A number of new window frames (500 by 1000 mm) made of pinewood, which were desired to be improved as regards the wood quality were freed of glass and possible hardware. The frames were then immersed into a large heated vessel containing linseed oil varnish, i.e. pure linseed oil with drier (siccative) added and an insecticide and fungicide. The linseed oil had a temperature of 250°C or slightly below. The frames were kept immersed for 10-20 minutes. They were then taken out of the bath and brought to a drying chamber where the air temperature was about 50°C and the air change was uniformly slow. The drier (siccative) added to the linseed oil comprised 0.07% lead 0.003% manganese and 0.004% calcium. The following naphthanates: 0.3% copper naphthanate and 0.3% zink naphthanate were added as insecticide and fungicide.

The finished frames displayed a marked improvement of the strength of the wood and the joints between the frame sections of which the individual frame is constructed, proved to be very compact. The frames displayed no tendency to warp (crookedness) and were entirely without fungus spores. Furthermore, the frames did not provide genial soil to the fungus spores.

### Example 2

It was desired to preserve and provide new strength to an article of prepared wood (an old piece of skirting board) which was attacked by dry rot and insects. The article was immersed in a bath of 180°C hot oil and kept under the surface of the oil for 20 minutes. At the end of this period the water evaporation from the article had ceased and there were only signs of the oil sizzling around the article. The bath which comprised linseed oil had been admixed with a drier (siccative) of 0.07% lead, 0.003% manganese and 0.004% calcium.

The following naphthanates: 0.3% copper naphthanates and 0.03 zink naphthanates were added as insecticide and fungicide.

After being taken out of the bath and excessive oil had dripped off and dried off, the article was left to dry in the open. The surface had dried after 48 hours. A corresponding article was impregnated in a similar manner but then placed in a heat chamber with air change and an average temperature of about 50°C. The latter article was dry and ready for use after 24 hours. Both articles were without warpings and resistant to both fungus and insect attacks.

### Example 3

A number of wooden articles of pinewood were formed to have dimensions almost corresponding to the dimensions of the worked end products. The degree of humidity of the starting articles was around 20%. The articles were immersed in a bath of 150°C hot linseed oil and were kept under the surface of the oil for 45 minutes. At the end of this period only signs of the oil sizzling around the articles were seen. The water evaporation had ceased before then.

Drier (siccative) in the form of 0.07% lead, 0.003% manganese and 0.004% calcium was added to the oil.

After taking the articles out of the bath, dripping off and drying off of excessive oil, the articles were dried in heating chamber with air change. The air was heated to about 80°C. The working took place after eight hours. It appeared that the oil had penetrated into the spring wood areas of the wood and therefore contributed in strengthening the structure of the wood. The working was carried out with conventional tools and machines. The degree of humidity had fallen to eight. The finished articles were without warpings (crookedness). The oil was admixed with fungicide preventing the articles from being attacked by fungus.

The invention may be varied in many ways without thereby deviating from the scope of its idea. The time spent by the articles in the linseed bath may thus be extended to several hours. Possibly, the drying time may be extended to more days.

## Claims

1. A method of quality improvement of wooden articles, such as improved preservation of wood through impregnation thereof, and where the impregnation is carried out by the wooden articles being immersed in a bath of hot linseed oil or similar vegetable oil, whereby the water present in the wood evaporates and diffuses through the wood and the oil while the hot oil simultaneously penetrates into the pores and cavities of the wood, whereupon the wooden articles are taken out of the bath and the oil oozed in is made to cure and thereby to stiffen the wood, **characterised** in that during the immersion of the wooden articles, the linseed oil bath has a temperature in the range of 145°- 250°C, preferably near 250°C, and that an insecticide and/or fungicide has been added to the linseed oil.

2. The method as claimed in claim 1, **characterised** in that drier (siccative) has been added to the linseed oil used.

3. The method as claimed in claim 1 or 2, **characterised** in that colour pigments have been added to the linseed oil used.

4. The method as claimed in claim 1, 2 or 3, **characterised** in that the treated articles are of old (used) wood.

5. The method as claimed in one or more of the claims 1-4, **characterised** in that the impregnation is carried out for a relatively short period, whereby the penetration of the linseed oil in the wooden material takes place to a rather slight depth.

6. The method as claimed in one or more of the claims 1-5, **characterised** in that after having been impregnated at the high temperature by the linseed oil, the wooden articles are subjected to a controlled drying (curing process) in heat chamber or autoclave.

7. The method as claimed in one or more of the claims 1-6, **characterised** by the linseed oil bath having a temperature of 175-245°C, during the immersion of the wooden articles.

8. The method as claimed in claim 7, **characterised** by the linseed bath having a temperature of 210-240°C, preferably 225-235°C, during the immersion of the wooden articles.

9. The method as claimed in one or more of the claims 1-8, **characterised** in that the wooden articles are kept immersed in the linseed bath for at least 10 minutes, preferably 15-60 minutes.

## Patentansprüche

1. Verfahren zur Qualitätsverbesserung von Holzgegenständen wie verbesserte Holzhaltbarkeit durch seine Imprägnierung, und wobei die Imprägnierung dadurch durchgeführt wird, daß die Holzgegenstände in ein Bad aus heißem Leinöl oder einem ähnlichen vegetarischen Öl eingetaucht werden, wobei das in dem Holz vorliegende Wasser verdampft und durch das Holz und das Öl diffundiert, während gleichzeitig das heiße Öl in die Poren und Hohlräume des Holzes eindringt, worauf die Holzgegenstände aus dem Bad herausgenommen werden und das eingesickerte Öl gehärtet wird und sich dabei das Holz versteift, dadurch gekennzeichnet, daß während des Eintauchens der Holzgegenstände das Leinölbad eine Temperatur im Bereich von 145 °C - 250 °C, vorzugsweise nahe bei 250 °C hat, und daß ein Insektizid und/oder Fungizid zu dem Leinöl zugegeben wurde.

2. Verfahren gemäß Anspruch 1, dadurch gekennzeichnet, daß ein Trockenmittel (Sikkativ) zu dem verwendeten Leinöl zugegeben wurde.

3. Verfahren gemäß Anspruch 1 oder 2, dadurch gekennzeichnet, daß Farbpigmente zu dem verwendeten Leinöl zugegeben wurden.

4. Verfahren gemäß Anspruch 1, 2 oder 3, dadurch gekennzeichnet, daß die behandelten Gegenstände aus altem (gebrauchtem) Holz sind.

5. Verfahren gemäß einem oder mehreren der Ansprüche 1-4, dadurch gekennzeichnet, daß die Imprägnierung während eines relativ kurzen Zeitraums durchgeführt wird, wobei das Eindringen des Leinöls in die Holzgegenstände in einer eher geringen Tiefe erfolgt.

6. Verfahren gemäß einem oder mehreren der Ansprüche 1-5, dadurch gekennzeichnet, daß die Holzgegenstände, nachdem sie bei der hohen Temperatur durch das Leinöl imprägniert worden sind, einer gesteuerten Trocknung (Härtungsverfahren) in einer Heizkammer oder einem Autoklav unterworfen werden.

7. Verfahren gemäß einem oder mehreren der Ansprüche 1-6, dadurch gekennzeichnet, daß das Leinölbad eine Temperatur von 175 °C-245 °C während des Eintauchens der Holzgegenstände hat.

8. Verfahren gemäß Anspruch 7, dadurch gekennzeichnet, daß das Leinölbad eine Temperatur von 210 °C-240 °C, vorzugsweise 225°C-235 °C, während des Eintauchens der Holzgegenstände hat.

9. Verfahren gemäß einem oder mehreren der Ansprüche 1-8, dadurch gekennzeichnet, daß die Holzgegenstände in dem Leinölbad während wenigstens 10 Minuten, vorzugsweise 15-60 Minuten, eingetaucht bleiben.

## Revendications

1. Procédé d'amélioration de la qualité d'articles en bois par imprégnation de ces derniers, tel que pour une meilleure conservation du bois, et dans lequel l'imprégnation est effectuée par immersion des articles en bois dans un bain d'huile de lin chaude ou d'une huile végétale analogue chaude, grâce à quoi l'eau présente dans le bois s'évapore et se diffuse à travers le bois et l'huile, tandis que l'huile chaude pénètre simultanément dans les pores et les cavités du bois, à la suite de quoi on sort les articles en bois du bain et on fait durcir l'huile qui s'y est infiltrée pour qu'elle rigidifie ainsi le bois, caractérisé en ce que, durant l'immersion des articles en bois, le bain d'huile de lin est à une température située dans la plage allant de 145° à 250° C, de préférence à une température proche de 250° C, et en ce qu'un insecticide et/ou un fongicide à été ajouté à l'huile de lin.

2. Procédé selon la revendication 1, caractérisé en ce qu'un agent séchant (siccatif) à été ajouté à l'huile de lin utilisée.

3. Procédé selon la revendication 1 ou 2, caractérisé en ce que des pigments de coloration ont été ajoutés à l'huile de lin utilisée.

4. Procédé selon la revendication 1, 2 ou 3, caractérisé en ce que les articles traités sont en bois âgé (bois usagé).

5. Procédé selon une ou plusieurs des revendications 1 à 4, caractérisé en ce que l'imprégnation est effectuée pendant une période de temps relativement courte, de manière que la pénétration de l'huile de lin dans le matériau en bois se fasse à une profondeur plutôt faible.

6. Procédé selon une ou plusieurs des revendications 1 à 5, caractérisé en ce que, après avoir été imprégnés à la température élevée par l'huile de lin, les articles en bois sont soumis à un séchage contrôlé (traitement de durcissement) dans une chambre chauffante ou un autoclave.

7. Procédé selon une ou plusieurs des revendications 1 à 6, caractérisé par le fait que le bain d'huile de lin a une température de 175 à 245° C, pendant l'immersion des articles en bois.

8. Procédé selon la revendication 7, caractérisé par le fait que le bain d'huile de lin a une température de 210 à 240° C, de préférence de 225 à 235°C, pendant l'immersion des articles en bois.

9. Procédé selon une ou plusieurs des revendications 1 à 8, caractérisé en ce que les articles en bois sont maintenus immergés dans le bain d'huile de lin pendant au moins 10 minutes, de préférence 15 à 60 minutes.
